# EUROPEAN PATENT SPECIFICATION

(11) **EP 0 320 083 B1**
(45) Date of publication and mention of the grant of the patent: **27.09.1995**
(21) Application number: 88306287.9
(22) Date of filing: 08.07.1988
(51) Int. Cl.: H01L 39/24, B03C 1/02

(54) **Purification apparatus for superconductor fine particles**
Reinigungsapparat für feine supraleitende Teilchen
Appareil de purification pour des particules fines supraconductrices

(30) Priority: 09.12.1987 JP 309473/87; 29.03.1988 JP 73363/87; 06.04.1988 JP 83025/87; 06.04.1988 JP 83026/87
(43) Date of publication of application: 14.06.1989
(62) Divisional of application: 93203438.2
(73) Proprietor: CANON KABUSHIKI KAISHA, Tokyo (JP)
(72) Inventor: Kishi, Fumio, Atsugi-shi Kanagawa-ken (JP); Akaike, Masatake, Atsugi-shi Kanagawa-ken (JP); Yamamoto, Keisuke, Atsugi-shi Kanagawa-ken (JP); Motoi, Taiko, Sagamihara-shi Kanagawa-ken (JP); Kaneko, Norio, Atsugi-shi Kanagawa-ken (JP); Iwatate, Fujio, Setagaya-ku, Tokyo (JP); Ohmi, Kazuaki, Yokohama-shi, Knanagawa-ken (JP); Kawasaki, Takehiko, Atsugi-shi, Kanagawa-ken (JP); Shinjou, Atsuko, 4-chome, Isehara-shi, Kanagawa-ken (JP)
(74) Representative: Beresford, Keith Denis Lewis

(56) References cited:
- WO-A-88/08619
- J. PHYS. E: SCI. INSTRUM., vol. 20, 6th October 1987, pages 1292-1293, GB; S. VIEIRA et al.: "A simple device for quick separation of high-Tc superconducting materials"
- APPLIED PHYSICS LETTERS, vol. 51, no. 23, 7th December 1987, pages 1954-1956, New York, US; M. BARSOUM et al.: "Use of Meissner effect to separate, purify and classify superconducting powders"
- PATENT ABSTRACTS OF JAPAN, vol. 13, no. 199 (C-594)[3547], 11th May 1989 & JP-A-1 22 359
- PATENT ABSTRACTS OF JAPAN, vol. 13, no. 211 (C-597)[3559], 17th May 1989 & JP-A-1 30 659
- PATENT ABSTRACTS OF JAPAN, vol. 13, no. 137 (C-582)[3485], 5th April 1989 & JP-A-63 302 966
- PATENT ABSTRACTS OF JAPAN, vol. 13, no. 187 (C-592)[3535], 2nd May 1989 & JP-A-1 15 158

## Description

The present invention relates to an apparatus and a method for purifying a superconductor fine particles. It enables desired superconductor particles to be obtained selectively from mixtures of fine particles of different diameters and comprised of superconductors, normal conductors or insulators having different critical temperatures and critical magnetic fields.

In recent years it has been discovered that by sintering ceramic materials with particular compositions there can be obtained a sinter that exhibits superconductivity (or is superconducting) at 77°K or above, in some instances near room temperature. However, the crystal structure and phase of these superconductors has not been sufficiently elucidated and usually they coexist with non-superconducting crystal phases.

It is very difficult to separate superconducting crystal phases from non-superconducting crystal phases where these phases coexist. Furthermore a technique of controlling heat treatment conditions has not been established that enables only superconducting crystalline materials to be formed. In recently available ceramic superconductors, there also often coexists a plurality of superconducting crystal phases which differ in their critical temperature or critical magnetic field. No method has been established for selectively separating the superconducting crystal phases having a particular desired critical temperature range and critical magnetic field range from amongst the various superconducting phases present.

In addition, superconductive sinter generally comprises a mass or aggregate of fine crystals and its superconductivity characteristics vary greatly depending on the state of the crystal grain boundaries. In order to produce a sinter having stable characteristics, the crystal grain boundaries must be made uniform. It has been proposed to produce a superconducting sinter of uniform crystal grain boundaries by re-sintering superconductor fine particles of uniform particle diameter. However, up to now no suitable method for classifying such superconductor fine particles of uniform particle diameter has been discovered, and only ordinary particle classification methods are available as described in from Funtai Kogaku Handobukku (Particle Technology Handbook) (edited by Koichi Iitani, Asakura Publishing Co). Ordinary particle classification methods involve screening by means of sieves having different opening sizes which are stacked up in order from those having the largest openings to enable classification to be carried out. A sedimentation method is known in which the terminal velocity at which particles in a fluid settle is used to carry out the classification.

However, in the screening method it is impossible to prepare screens whose sizes are several micrometres or below, thus preventing particles of small diameter from being classified. Furthermore, it is often the practice to apply a load to the fine particles in order to produce a pressure tending to force them through the openings in the screen. This practice gives rise to the problems that classification cannot be carried out in a vacuum, as would otherwise be preferred because of its greater precision. In the sedimentation method described above, the settling velocity depends both on the diameter of the particles and on the specific gravity thereof, and accurate classification cannot be achieved. Furthermore, in liquid phase sedimentation methods it is laborious to separate fine particles from liquid and in general the settling velocity is so low that the time required for classification is very lengthy. The method also suffers from the problems that it is inherently not a vacuum method.

A method for separating superconducting particles from non-superconducting particles by means of magnetic levitation is disclosed in a paper by S Vieira et al, "A Simple Device for Quick Separation of High-Tc Superconducting Materials", J. Phys. E: Sci Instrumen. 20 (1987) 1292-1293. Another magnetic separation method is disclosed in a paper by Barstoum et al, "Use of the Meissner Effect to Separate, Purify and Classify Superconducting Powders", Appl. Phys. Lett. 51(23), 7 December 1987, page 1954. Patent Publication WO88/08619 discloses a method of separating superconductive materials from other materials by allowing the material to fall and applying a magnetic field to the falling material.

The apparatus and method of this invention are defined in the accompanying claims.

Forms of the above defined apparatus enable superconductor fine particles to be separated and purified when they are present as a powder containing other particles. Further forms of the invention enable superconductor fine particles to be classified and purified according to the desired characteristics, when there is present in a powder a plurality of such fine particles having different characteristics e.g. particle diameter, critical temperature and critical magnetic field.

Various forms of the invention will now be described, by way of example only, with reference to the accompanying drawings.

### BRIEF DESCRIPTION OF THE DRAWINGS

Figs. 1, 4, 7, 12, 13, 14, 15, and 16 each illustrate schematic constitution of an example for the purification apparatus for superconductor fine particles according to the present invention;
Fig. 2 is a graph showing an X-ray diffraction 25 pattern of a superconductor containing impurities;
Fig. 3 is a graph showing an X-ray diffraction pattern of a purified superconductor;
Fig. 5 is a graph showing temperature dependency of the electric resistance of a superconductor;
Fig. 6 illustrates constitution of another example of a magnet and a partition panel part of the apparatus of the present invention;
Fig. 8 illustrates constitution of another example of a powder-feeding means in the apparatus of the present invention;
Figs. 9 and 10 each illustrate constitution of another example of a means for applying magnetic field in the apparatus of the present invention;
Fig. 11 illustrates constitution of another example of a powder-collecting means in the apparatus of the present invention;
Figs. 28 and 29 respectively illustrate a block diagram and a time chart of a controlling system in the apparatus of the present invention;
Figs. 30 and 31 respectively illustrate a block diagram and a time chart of another controlling system in the apparatus of the present invention.

### DETAILED DESCRIPTION OF THE PREFERRED EMBODIMENTS

The present invention is based on the utilization of the Meissner effect which is attributable to magnetic properties inherent in superconductors.

The Meissner effect is meant to be the effect that the superconductor fine particles become perfectly diamagnetic when a magnetic field is applied to the fine particles at the temperature at which the superconductor fine particles exhibit superconductivity. More specifically, at the abovementioned temperature, application of a magnetic field by means of a magnet to the powder containing superconductor fine particles produces repulsion to the magnet owing to the Meissner effect with respect to those having a particle diameter of about 0.01 µm or more. On the other hand, no repulsion is produced since the Meissner effect is not brought about with respect to those having a particle diameter less than that and the fine particles of normal conductors or insulators.

According to this principle it is possible to separate and purify with a high precision only the superconductor fine particles from among the powder mixed with normal conductors or insulators.

For example, a flow of powder to be purified, mixed with normal conductors, insulators, etc. is formed, and a magnetic field with a strength by which the superconductivity can be effectively utilized is applied to the powder to be purified, under the temperature of the degree at which the superconductor fine particles in the powder to be purified exhibit the superconductivity, so that the repulsion produced as a result owing to the Meissner effect causes positional separation of the flow of the superconductor fine particles in the powder to be purified, from the flow of the particles other than the same, thus effecting the purification.

The locus of the flow of a superconductor-containing fine particle that shifts according to Meissner effect depends on the proportion of the superconductor contained in the fine particle. This is because the force by which the superconductor fine particle is moved is produced by Meissner effect. Namely, even if the superconductors have the same particle diameters, the repulsion becomes small when the proportion of the superconductors is small. In other words, the low purity thereof results in a small change in the locus of the flow of particles.

For example, in instances where a magnetic field having the distribution such that the magnetic flux density becomes smaller from a lower part toward an upper part is applied, the particles having a small proportion of superconductors may be given small Meissner effect, resulting in a small height of floating. On the contrary, the particles having a large proportion of superconductors can float higher. The floating height depends on the balance between the weight of particles and the greatness of the Meissner effect.

By selectively collecting portions at a certain height of the thus floated superconductor fine particles, it is possible to take out only the superconductor fine particles having desired purity, i.e., desired values for the proportion of superconductors.

Here may be used any means for forming the flow of powder in a gaseous carrier medium along a path, including, for example, a means for directly blowing a carrier gas to the powder.

The carrier gas used in the apparatus of the present invention may include, for example, helium gas. Also preferred is a gas that may not liquified even at a temperature sufficiently lower than the critical temperature of the superconductors.

The means for applying a magnetic field to the flow of the above powder include, for example, a permanent magnet and an electromagnet, which magnets may have any shape so long as there can be applied a magnetic field by which the superconductor fine particles can deflect their flying path. Accordingly, it may include plate-shaped, column-shaped or concave-shaped magnets, or those arranged with a plurality of these magnets.

In instances where a desired particle diameter or particle size distribution is to be obtained, various types of classifying means can also be used in combination according to the range of the desired particle diameter. However, since the Meissner effect for the effective purification can be obtained usually in respect of the superconductor fine particles having a particle diameter of 0.01 µm or more, the fine particles having a particle diameter of 0.01 µm or more and the fine particles having a less particle diameter can be readily classified, which have ever been classified not easily by conventional classification methods.

It is also possible to carry out classification of particles of the particle diameters other than that. More specifically, if powder having uniform specific gravity are treated in the apparatus of the present invention, the difference in flying distance or floating height of the particles owing to the carrier gas, for example, depends on their particle diameter. Therefore, they may be collected selectively by zones, so that it becomes also possible to classify the superconductor fine particles included in a desired particle diameter range from among the superconductor fine particles having a particle diameter of 0.01 µm or more.

To carry out the powder classification with higher precision in the apparatus of the present invention, a partition means having one or plural slit(s) may preferably be provided additionally in the same apparatus.

In the apparatus of the present invention, superconductor fine particles having a desired critical temperature range or critical magnetic field range can also be obtained from among the powder in which a plurality of superconductor fine particles each different in the critical temperature (superconductive transition temperature) or critical magnetic field (superconductive transition magnetic field).

For example, in instances where the superconductor fine particles having a desired critical temperature range are to be obtained in the above purification apparatus, the above purification apparatus may be operated while appropriately selecting the temperatures of a powder storing vessel, a carrier gas, a powder flow path, etc. according to the desired critical temperature range.

Also in instances where the superconductor fine particles having a desired critical magnetic field range are to be obtained, the above purification apparatus may be operated while appropriately selecting the magnetic field applied to the powder to be purified, according to the desired critical magnetic field range.

In the apparatus of the present invention, it is further possible to obtain only the powder having a desired specific gravity, not to speak of the above purification and classification of the superconductor fine particles.

More specifically, if the powder have a uniform particle diameter, the difference in flying distance or floating height of the powder owing to the carrier gas and the degree of changes in the flow direction of superconductor fine particles owing to the application of a magnetic field depend on their specific gravity. Therefore, they may be selectively collected by zones, so that it becomes also possible to separate only the superconductor fine particles having a desired specific gravity.

The above purification apparatus for superconductor fine particles of the present invention will be described below by giving several preferred embodiments.

A first embodiment of the apparatus of the present invention is characterized by having a means for horizontally ejecting powder containing superconductor fine particles to form a flow of the powder, a partition means horizontally provided, having one or plural slit(s) at the position with a specified distance from an ejecting outlet, and a means provided beneath said respective slit(s), for applying a magnetic field in the vertical direction to the flow of said powder

According to the present embodiment, the powder to be purified containing superconductor fine particles maintained to a temperature at which their superconductivity can be sufficiently exhibited are horizontally ejected from a nozzle or the like together with a carrier gas, whereupon the powder particles larger in particle diameter and heavier among the powder to be purified begin to fall at a position near to the above nozzle, and the particles smaller in particle diameter and lighter among them begin to fall at a position far from the above nozzle, so that the groups of the falling powder particles form the particle size distribution in the horizontal direction. Classification can be carried out by selectively separating them by the partition means horizontally provided, having one or plural slit(s) at the position with an appropriate distance from the nozzle. Here, the various conditions such as the kind of the above-mentioned carrier gas, the flow rate, the flow quantity, the slit width may be appropriately selected according to the desired particle diameter range.

Only the superconductor fine particles can also be separated by providing a plate-shaped magnet beneath the above slit, having a width and shape sufficient for making purification under the above temperature, in a vertical state or a state slightly inclined than vertical, applying the magnetic field previously mentioned to the powder to be purified that have been classified and passed the slit as described above to let the powder fall in the vicinity of the plate-shaped magnet, under the temperature previously mentioned, to change the falling locus of the superconductor fine particles in the powder to be purified, and collecting them by use of a collecting means each provided at the falling position of the superconductor fine particles and at the falling position of the other fine particles. Thus, the apparatus of the present embodiment can carry out the purification and classification simultaneously.

In the above apparatus, the means for applying a magnetic field may be any of a permanent magnet and an electromagnet, without any particular limitation also in its shape. However, when, for example, a sheet of the above plate-like magnet is constituted of a plurality of electromagnets to give a means for applying magnetic fields that can repeat on-off in succession in the powder-falling direction and with a specified period, the falling locus of the superconductor fine particles can be changed with good efficiency to bring about the advantages such that the purification process can be simplified. To attempt to further simplify this purification process, a plate of non-magnetic material may be provided on the surface of the magnet and may be vibrated (as exemplified by an ultrasonic vibration plate), thus making it possible to smooth the flow of powder.

A second embodiment of the apparatus of the present invention is characterized by a means for floating the powder containing superconductor fine particles, in a carrier-gas flow path, a means for applying a magnetic field that may move the superconductor fine particles in the vertical direction to the carrier gas flow formed by the first-mentioned means, and a partition means vertically provided, having one or plural slit(s) at the position facing said magnetic field applying means.

According to the present embodiment, the powder containing superconductor fine particles are floated by the floating means using a carrier gas, so that, if the powder have a uniform particle diameter, the powder having a smaller specific gravity float higher and the powder having a larger specific gravity float only up to a lower position. Accordingly, the purification and separation can be simultaneously carried out by applying a magnetic field to the floating powder, separating selectively to the outside of the carrier gas flow only the superconductor fine particles from among the powder by the repulsion owing to the Meissner effect, through means of a partition panel provided with one or plural slit(s) and according to the height of the slit(s), and collecting the particles using a collecting means provided at the outside of the carrier gas flow.

Here, the floating means may be any means so long as it is a means capable of blowing the powder by use of the carrier gas, and may include, for example, a means for directly blowing the carrier gas to the powder, a means for putting the powder in a container and introducing the carrier gas in that container, a means for allowing the powder to fall from a container and blowing the carrier gas to that falling powder, and a means for making suction from the direction of the magnetic field applying means.

The magnetic field applying means may also be any of a permanent magnet and an electromagnet also in the present embodiment, without any particular limitation in its shape. When the magnet comprises, for example, an electromagnet to give a means for applying a magnetic field that can repeat on-off synchronously with the powder floating means and with a specified period, the classification can be carried out more precisely.

In this instance, the respective sections can be synchronized by electrical control with use of a controlling system as shown in Fig. 28. In Fig. 28, the numeral 101 denotes a synchronizing computer; 102, a shutter to open and close an inlet (Position A exemplified in Fig. 14 and Fig. 15 of the apparatus of an Example described later) for injecting a carrier gas for blowing up the powder; 103, a shutter fitted to an inlet (Position B exemplified in Fig. 14 and Fig. 15 of the apparatus of an Example described later) for introducing the superconductor fine particles discharged from the carrier-gas flow path by the repulsion owing to the Meissner effect from among the given floated fine particles; 104, an electric source for the magnet; 105, the electromagnet (which is provided at Position M exemplified in Fig. 14 and Fig. 15 of the apparatus of an Example described later) that produces the magnetic field necessary for purifying the superconductor fine particles owing to the Meissner effect.

The above shutters and magnet are driven by being synchronized as shown in Fig. 29. In Fig. 29. the abscissas indicate the time, and the ordinates indicate the driving pulse in respect of the actuation of the shutters 102 and 103, and the electric current to be flowed in respect of the magnet 105. The shutters 102 and 103 turn "open" by the rise of the pulse and turn "close" by the decay of the pulse.

First, the shutter 102 turns "open" to bring the powder particles to float in the carrier-gas flow path together with the carrier gas. The shutter 103 turns "open" when the time t₁ lapses and the floating positions have been settled for each particle diameter, and at the same time the magnet turns "on". Thereafter, during the time t₂, the superconductor fine particles are discharged from the carrier-gas flow path through the introducing inlet. Thereafter the shutters 102 and 103 turn "close" and the magnet turns "off". After the time t₃ lapsed and the non-superconductor particles having remained in the carrier-gas flow path have fallen, the shutter 102 again turns "open", thus repeating the above operations.

In an instance where a means for collecting non-superconductors is provided (exemplified in Fig. 15 of the apparatus of an Example described later), equipped is a shutter 106 (at Position C in Fig. 15). A block diagram and a time chart in a controlling system for that instance are shown in Fig. 30 and Fig. 31, respectively. Operations are the same as described above. The shutter 106 turns "close" when the shutter 102 is "open", and the shutter 106 turns "open" when the shutter 102 is "close".

In the above apparatus, the various conditions such as the type of the above carrier gas, the flow rate, the flow quantity, the width of the slit may be suitably selected according to the desired particle diameter range.

As described previously, the ultrasonic vibration plate that may be provided on the surface of the magnet in the first embodiment of the present invention employing a piezoelectric material (such as ZnO, AlN and PZT). There is no particular limitation in the frequency of the vibration, but in general it may range approximately from 1 Hz to 20 kHz.

As having described above, employment of the apparatus of the present invention makes it possible to simultaneously and readily carry out the purification, classification and separation of superconductor fine particles having the desired purity, particle diameter, critical temperature range and critical magnetic field range from among the powder to be purified, and the apparatus used in the process can be of small size and simple, with the course of the process capable of being visually observed. Moreover, the process can be carried out under a low pressure, and yet the above process is proceeded while forming the flow of the powder to be purified. Accordingly, a large quantity of powder can be purified in a high rate and high precision.

The apparatus of the present invention is also very useful in enhancing the purity of a superconductive sinter that contains impurities. More specifically, since the present invention can carry out the purification and classification in the order of a µm unit, the sinter can be very finely grounded and purified to the extent such that a superconductivity part and an impurity part may not coexist in its one fine particle. As a result, there can be obtained superconductive powder with high purity.

In the apparatus of the present invention, it is also further possible to obtain superconductor fine particles having uniform specific gravity, and thus possible to obtain superconductors with less intermixing of superconductors having different composition.

### EXAMPLES

The present invention will be described below in greater detail by giving Examples and also with reference to the drawings.

### Example 1

Fig. 1 illustrates an example of the apparatus of the present invention. The numeral 9 indicates superconductor fine particles having relatively large particle diameter; 10, superconductor fine particles having relatively small particle diameter of about 0.1 µm or less; and 7 and 8, non-superconductor fine particles having relatively large particle diameter and non-superconductor fine particles having relatively small particle diameter. In the present Example, the superconductive material to be classified and purified is YBa₂Cu₃O_{7-δ} (0 ≦ δ ≦ 0.5). Y₂O₃, BaCO₃ and CuO were mixed in a ratio of Y : Ba : Cu = 1 : 2 : 3, and the mixture was treated by heating for 2 hours at 950°C in an atmosphere. The X-ray diffraction pattern obtained here is shown in Fig. 2. In Fig. 2, the peaks in the intended superconductor YBa₂Cu₃O_{7-δ} are indicated by "S". As will be clear from this figure, this sample contains a non-superconductor.

The mixture was ground in a mortar, and thereafter the settling velocity was measured in toluene to reveal that the settling velocity differs depending on the particle diameter, but the particles having the same particle diameter as a whole settled substantially in the same velocity. Accordingly, the superconductors and the impurity non-superconductors are considered to have substantially the same specific gravity.

First, powder containing superconductor fine particles and a carrier gas (as exemplified by He gas) having a temperature not higher than the critical emperature are mixed to make a mixed powder 1. This is ejected from an opening 2. The ejecting rate is selected depending on the specific gravity of powder or the particle diameter range as desired. The position of slits 11a and 11b of a partition panel 3 is made movable, and the width of the slits is selected by the particle diameter range as desired. Fine particles having a larger particle diameter are transported near the opening 2, and smaller fine particles having a smaller particle diameter, up to a distant place by the carrier gas. The powder having uniform particle diameter pass the slits and then fall by gravity, but at this time, because of a plate-shaped permanent magnet, the superconductor fine particles 9 having relatively large particle diameter become apart from the surface of the magnet to pass over a partition panel 4a to fall. However, it may not occur that normal conductors, i.e., the fine particles 7 of non-superconductor (including conductors, semiconductors and insulators) pass over the partition panel 4a. The superconductor fine particles passed over the partition panel 4a are collected by a collection receptacle 6a. Similarly, the superconductor fine particles 10 having relatively small particle diameter are also separated from the non-superconductor fine particles 8 by a permanent magnet 5b and a partition panel 4b, and collected in a collection receptacle 6b.

In the present Example, the classification and purification are carried out under the following conditions. In Fig. 1, the mixed powder 1 is ejected from the opening 2 at a flow rate of about 200 ml/min with use of the carrier gas comprising He gas. The He gas is beforehand cooled to a temperature of 70 K or less by use of a cooling unit (not shown). The slit 11a has a space of 3 mm, and the slit 11b, 4 mm. The distance from the opening 2 to the slit 11a is 50 cm, and that from the opening 2 to the slit 11b, 150 cm. The permanent magnets are all comprised of Sm-Co and cooled to a temperature of 77 K using a a cooling unit (not shown). The partition panels 4a and 4b protrude by 4 mm from the surface of the magnets 5a and 5b. Under the working conditions as described above, superconductors were able to be collected from about 5 g of raw material powder in the collection receptacle 6a in an amount of about 2.5 g, and in the collection receptacle 6b, about 2 g. The powder in this collection receptacle showed the X-ray diffraction pattern as shown in Fig. 3, resulting in disappearance of all the diffraction peaks of the non-superconductor fine particles in Fig. 2. Thus it was able to confirm that the present apparatus can make purification of superconductors. An electron microscope also revealed that superconductors of about 100 to 200 µm in particle diameter have been collected in the collection receptacle 6a, and those of about 10 to 50 µm in particle diameter, in the collection receptacle 6b, thus confirming the effect of classification.

### Example 2

In the case when the powder containing superconductor fine particles have a large particle size distribution and at the same time contain large particles of about 100 µm or more in particle diameter, the opening 2 is made to have the shape of a nozzle, and powder flow is ejected from the nozzle-shaped opening 2 so that the ratio of the pressures of the carrier gas before and after passing the nozzle-like opening 2 may be 10 or more. This operation enables the classification of the superconductor fine particles with a high efficiency like in Example 1 even if the powder contains those having a particle diameter of about 100 µm or more.

### Example 3

It may often occurs that superconductor phases having different critical temperatures coexist if ceramics having the composition such as YBa₂Cu₃Oₓ (x = 6.00 to 7.00) or Bi₂ (Sr, Ca)₃ Cu₂O₁₂₋ₓ (x > 0) are sintered under the same conditions. In such an instance, used is an apparatus having functions as shown in Fig. 4.

In Fig. 4, the numeral 7a indicates non-superconductor fine particles having relatively large particle diameter; 8a, non-superconductor fine particles having relatively small particle diameter; and 9a, 9b, 10a and 10b each, superconductor fine particles, where 9 indicates a higher critical temperature than 10, and a indicates those having relatively large particle diameter, and b, those having relatively small particle diameter.

The temperature dependence on the electric resistance of the superconductors used as samples of the present invention is shown in Fig. 5. As will be seen from Fig. 5, there exists a crystal phase that exhibits superconductivity at 107 K or less.

In a mortar, about 10 g of raw material powder is ground, and this is ejected from an opening 2 of 5 mm in diameter at a flow rate of about 300 ml/min by using He gas cooled to about 60 K as a carrier gas. Sm-Co magnets 5a and 5b at the upper stage are beforehand cooled to 50 K by means of a cooler (not shown) and Sm-Co magnets 5c and 5d at the lower stage are similarly beforehand cooled to 90 K. The partition panels 4a and 4b at the upper stage protrude by 4 mm from the surface of the magnets and the partition panels 4c and 4d at the lower stage protrude by 3 mm. As a result, superconductors (critical temperature: 107 K) having a particle diameter of about 100 to 400 µm were collected in the one collection receptacle 6a and those having a particle diameter of about 30 to 50 µm were collected in the other collection receptacle 6b in an amount of about 0.05 g and 0.08 g, respectively. On the partition panels 4c and 4d, also collected were 3 g and 5 g, respectively, of superconductors haing a critical temperature of 80 K. Meanwhile, the slits 11a and 11b are both 5 mm in width, and the slit 11 is 70 cm distant and the slit 11b is 200 cm distant, from the opening 2.

### Example 4

In Examples 1 to 3, the magnets and the partition panels at the bottom parts thereof, as exemplified by the magnets 5a and 5b and the partition panels 4a and 4b in Fig. 1 had the shapes of flat plates. The partition panels 4a and 4b are made to have the shapes having edges fitted on their both ends as shown in Fig. 6, and in some instances the partition panels are made continuously movable according to a belt conveyor system. This makes it possible to make separation of a large quantity of powder.

### Example 5

In the instances where the powder containing superconductor fine particles have relatively uniform grain size and no further classification is required as in Examples 1 to 4, no carrier gas is required, and the superconductor fine particles can be separated by allowing the powder to fall on a magnet 5 as shown in Fig. 7.

More specifically, the powder is allowed to fall from a container 12 holding the powder containing superconductor fine particles, and the powder may be brought to slip down the surface of the magnet 5 by appropriately selecting the inclination of the magnet 5 from a vertical position according to the particle diameter of the powder, so that only the superconductors 9 kept apart from the magnet surface pass over the partition panel owing to the Meissner effect and are collected in a collection receptacle 6.

### Example 6

As shown in Fig. 8, powder is allowed to fall from the container 12 holding the superconductors 9 to make the apparent shape of the powder falling on a slip board 13 to be of thin plate, to which a carrier gas is blown through a gas-introducing pipe 14. The classification of the superconductor fine particles can be carried out in the same manner as in Example 1 except for transporting the powder in this manner.

### Example 7

In Examples 1 to 5, the means for applying the magnetic field is constituted of a plurality of electromagnets 5I, 5II, 5III, ... and 5n as shown in Fig. 9, so that the on-off of the above electromagnets may be repeated (in the order of 5I → 5II → 5III → ... 5n → 5I) by a means (not shown) for controlling the application of magnetic fields, in succession in the falling directions of from 5I to 5n and with an appropriate period. This makes it possible to attempt to simplify the purification process and separate a large quantity of powder.

The period of the on-off of the magnetic fields may be selected according to the velocity of the powder flow, and also the magnetic fields may be made stronger in succession from 5I toward 5n.

### Example 8

In Examples 1 to 5 and 7, provided is a vibration plate that ultrasonically vibrates by use of an ultrasonic oscillator (not shown) as shown in Fig. 10. This makes it possible to prevent the powder to be purified from being deposited on the magnets, attempt to make efficient the purification process, and separate a large quantity of the powder.

### Example 9

In instances where the powder containing superconductor fine particles have relatively a uniform particle diameter so that no further classification may be required, a collecting means as shown in Fig. 11, may be provided after the same classification and purification as in Example 1, so that the superconductor fine particles can be separated according to the difference in the specific gravity.

In Fig. 11, the numeral 19a denotes superconductor fine particles having relatively high specific gravity; 19, superconductor fine particles having relatively low specific gravity; and 7, non-superconductor fine particles, where all of these fine particles have substantially the same particle diameter.

The collecting means in the present embodiment comprises passages 18a and 18b and superconductors collection receptacles 6a and 6b, and is constituted such that the powder to be purified fall on the slant of a magnet 5, and the non-superconductor fine particles 7 in the powder continue to come into contact with the slant until they slip down in an impurities receptacle 17.

It is also constituted such that the superconductor fine particles 19b having relatively light specific gravity become greatly apart from the magnet 5 owing to the magnetic field applied, and the superconductor fine particles 19a having relatively heavy specific gravity are not so much apart from it so that the distribution of the flows according to the specific gravity can be formed.

It is also constituted such that each of the superconductor fine particles 19a and 19b in that distribution can be collected by superconductors collection receptacles 6a and 6b through the passages 18a and 18b.

The distance of the passages 18a and 18b from the magnet 5 in this apparatus and the inclination of the magnet 5 may be appropriately selected to find an optimum value according to the desired particle diameter and specific gravity. To carry out the classification and separation with further precise particle diameter and specific gravity, the passages 18a and 18b may be made to have a narrower width and the number of the passages may be increased.

### Example 10

If the spacing of the slits become broader, it can be contemplated, for example, in Fig. 1 that the non-superconductors pass over the partition panels 4a and 4b to mix into the collection receptacle. In such an instance, a flow-deflecting device 1 (as exemplified by a baffle) may be provided, so that the precision of the classification and purification can be improved.

### Example 11

The apparatus illustrated in Fig. 13 comprises a container 20, a diaphragm 21, a partition panel 3, a nozzle 1, and a funnel 23. The inside of the container is kept at about 70 K, and its lower part is filled with liquid nitrogen. The upper part thereof is filled with helium gas blown in from the nozzle together with sample powder.

The sample powder blown out from the nozzle falls from slits 11a, 11b and 11c corresponding to the respective superconductor to enter into the liquid nitrogen. Magnets 5a, 5b and 5c are provided in the vicinity of the powder-falling orbital path, and the superconductor fine particles are deflected in their orbital path by the repulsion owing to the Meissner effect and gathered in saucers 6a, 6b and 6c. The non-superconductor particles fall straight near the magnets and selected and separated from the superconductors.

In the present Example, the heat capacity of the liquid is larger by far than that of the gas so that the samples which fell into the liquid immediately come to have the same temperature as the liquid. Thus, this is characterized by having good precision for the temperature at the time of purification.

In the above Example, used magnets are all permanent magnets, but the magnetic fields may be applied to the powder by use of electromagnets to obtain quite the same effect. The slits are provided on the partition panels 3 at three points, but the slits may be made small in width and large in the number to effect precise classification of particle diameter. There are no particular limitations in the width and number of the slits. Alternatively, a vessel that can be moved by a belt conveyor or the like may be used in place of the slits, and this may, for example, be moved in the direction perpendicular to the paper surface of Fig. 13, and thereafter may be allowed to fall on the magnet areas.

Moreover, it is needless to say that the particle size distribution of the superconductor fine particles collected in the collection receptacle 6 may not be affected at all even if there is a great difference in the specific gravity between the superconductors and non-superconductors.

### Example 12

Fig. 14 is a schematic view illustrating another example of the apparatus of the present invention. In Fig. 14, the numeral 38a denotes superconductor fine particles having relatively large particle diameter; 39a, superconductor fine particles having a particle diameter of about 0.1 µm or more but a relatively small particle diameter; and 37a and 37b, non-superconductor fine particles.

The floating means in this Example comprises a powder container 31, a opening 32 and a carrier gas ejector (not shown). The magnetic field applying means comprises a magnet 36.

This apparatus is so constituted that the powder to be purified contained in the powder container 31 can be floated by the carrier gas from the powder container 31 to a vertical passage 33 through the opening 32. The fine particles 37a and 38a having relatively large particle diameter among the powder floated in the vertical passage 33 float only up to a lower position, but the superconductor fine particles 37a and 38b having relatively small particle diameter float up to a higher position. In this Fig. 14, all the superconductor fine particles and non-superconductor fine particles are assumed to have substantially constant specific gravities. The ejection rate at this time may be selected according to the specific gravity of the powder or the desired particle diameter range. The position, width and number of the vertical passage 33 and horizontal passages 34a and 34b may also be selected according to the desired specific gravity and particle diameter.

The apparatus is further so constituted that once a magnetic field is applied by a magnet 36 to the powder inside the vertical passage 33 which have floated to different heights depending on the particle diameter, the respective superconductor fine particles 38a and 38b move to the respective horizontal passages 34a and 34b by the action of the repulsion caused by the Meissner effect, and are collected in the collection receptacles 35a and 35b for the respective superconductor fine particles.

It is also so constituted that the non-superconductor fine particles 37a and 37b staying inside the vertical passage 33 fall into the powder container 31 by stopping ejecting the carrier gas or by turning down the gas.

Employing this apparatus makes it possible to simultaneously and readily carry out the classification-separation according to the particle diameter and/or specific gravity by floating the powder with use of a carrier gas, and the purification by applying the magnetic field to the powder.

In regard to the flow rate of the carrier gas and the driving timing t₁, t₂ and t₃ previously mentioned, the flow rate is 300 ml/min; t₁, 20 seconds; t₂, 5 seconds; and t₃, 1 minute in instances where, for example, the superconductor fine particles to be classified contains even the fine particles of about 1 to 3 µm in particle diameter.

In instances where the particles having a relatively large particle diameter of about 10 to 30 µm are classified, the flow rate is 1 lit/min; t₁, 20 seconds; t₂, 5 seconds; and t₃, 20 seconds, in approximation, which are typical values.

### Example 13

Fig. 15 is a schematic view illustrating an apparatus constituted by providing in the apparatus shown in Fig. 14 an impurities collection receptacle 39 and a closing flap 40, and arranging the opening 32 in the horizontal direction.

This apparatus is so constituted that when the non-superconductor fine particles 37 and 38 staying inside the vertical passage 33 are allowed to fall by stopping ejecting the carrier gas or by turning down the gas, they fall into the impurities collection receptacle 39 if the closing flap 40 is opened. Accordingly, the non-superconductor fine particles 37 and 38 may not return to the inside of the powder container 31 to enable the purification with good efficiency. Since moreover the direction of flow of the carrier gas containing the powder greatly changes, the powder tend to be uniformly distributed inside the vertical passage 33.

The flow rate of the carrier gas and the values for t₁, t₂ and t₃ are the same as in the case of Example 12.

### Example 14

In the case when the powder containing superconductor fine particles have a large particle size distribution and at the same time contain large particles of about 100 µm or more in particle diameter, the opening 2 of the apparatus illustrated in Fig. 14 or Fig. 15 is made to have the shape of a nozzle, and powder flow is ejected from the nozzle-shaped opening 2 so that the ratio of the pressure of the carrier gas before and after passing the nozzle-like opening 2 may be 10 or more. This operation enables the classification of the superconductor fine particles with a good efficiency like in Example 1 even if the powder contain those having a particle diameter of about 100 µm or more.

### Example 15

Fig. 16 illustrates an apparatus constituted by providing ultrasonic vibration plates 41a and 41b respectively at the bottom surfaces of the horizontal passages 34a and 34b of the apparatus illustrated in Fig. 14. or Fig. 15. In this apparatus, there is no friction resistance between the superconductor fine particles having moved from the vertical passage 33 to the horizontal passages 34a and 34b, and the bottom surfaces of the horizontal passages 34a and 34b, so that the superconductor fine particles can be efficiently transported to the collection receptacles 35a and 35b without stagnating on the way of the horizontal passages 34a and 34b.

### Example 16

In the apparatus shown in Fig. 14, Fig. 15 and Fig. 16, the magnet 36 was made to comprise an electromagnet, and the electromagnet was so provided that it can repeat on-off with a certain period while being synchronized with the powder-floating means by using a means (not shown) for controlling the application of magnetic fields. More specifically, the magnet was so provided that the magnetic field may be applied after lapse of an appropriate time by which the particle size distribution of the powder formed in the vertical direction inside the vertical passage comes to a steady state after ejection of the carrier gas, and further that this operation may be repeated with a specified period.

Employment of such an apparatus further improves the precision in the classification of the superconductor fine particles.

Also, using the apparatus shown in Fig. 14, about 5 g of powder (showing the same X-ray diffraction pattern as in Fig. 2) containing the superconductor fine particles obtained in the same manner as in Example 1 were added to the flow of a carrier gas of a temperature not higher than the critical temperature (He gas; 70 K or less), and this was ejected from the opening 32 at a flow rate of about 200 ml/min. The horizontal passage 34a was made to be 4 mm in width, and the horizontal passage 34b, 3 mm in width. The horizontal passage 34a was also made 5 cm apart from the opening 32, and 10 cm apart from the horizontal passage 34b.

Used for the magnet 36 was a permanent magnet (Sm-Co), and the inside of the apparatus was cooled to 77 K by a cooling means (not shown) to carry out the process.

With respect to about 5 g of the raw material powder the process of the present invention was carried out. As a result, it was able to collect about 2.5 g of superconductor fine particles in the collection receptacle 5a, and about 1.3 g of superconductor fine particles in the collection receptacle 5b.

The X-ray diffraction pattern of the superconductor fine particles in the collection receptacles 35a and 35b resulted in the same as in Fig. 3.

From these results, it was able to confirm that the apparatus of the present invention can make purification of superconductors in good precision.

Observation of the superconductor fine particles in the collection receptacles 35a and 35b using an electron microscope also revealed that the fine particles in the collection receptacle 35a had a particle diameter of about 100 to 200 µm, and the fine particles in the collection receptacle 35b, about 10 to 50 µm. From these results it was able to confirm that the apparatus of the present invention can make classification of superconductors having a very small particle diameter.

## Claims

1. Apparatus for purifying superconductor fine particles comprising means for cooling powder to be purified and containing the fine particles to below its critical temperature, means (2; 32) for forming a flow of the powder along a path, partition means having a plurality of openings (11a, 11b ; 34a, 34b) at different spaced-apart locations along the path for receiving particles of different properties, and means (5a, 5b ; 36) for applying a magnetic field to the flow of the powder to separate the fine particles by means of their superconductivity, characterised in that:
(a) the powder flow forming means is arranged to cause the powder to flow in a gaseous carrier medium along the path so that particles of different size separate according to their size and mass as they travel along the path; and
(b) the locations at which the openings (11a, 11b ; 34a, 34b) are provided are where gravitationally induced separation of particles of different sizes has taken place.

2. Apparatus according to claim 1, wherein the means for forming the flow of powder is arranged to blow the powder in a horizontal direction, the partition means is horizontally directed and has a plurality of openings at different distances from the blowing means, and means is provided beneath the respective openings for applying a magnetic field to the powder as it travels along the path.

3. Apparatus according to claim 2, wherein the blowing means comprises a nozzle.

4. Purification apparatus according to claim 2, wherein the magnetic field providing means comprises first magnets located relatively close beneath the respective openings and cooled to a first relatively low temperature and second magnets for receiving material that has passed from the first magnets and located at a relatively greater distance beneath the respective openings, the second magnets being cooled to a relatively high temperature, the arrangement being such that only material whose critical temperature for superconductivity is greater than the second temperature passes the second magnets.

5. Apparatus as claimed in claim 2,3 or 4, wherein there is provided beneath a respective opening a baffle facing oppositely to the blowing direction of the powder for directing the powder towards the magnetic field applying means.

6. The apparatus of any preceding claim, wherein the means for applying a magnetic field comprises a permanent magnet.

7. The apparatus of any of claims 1 to 5, wherein the means for applying a magnetic field comprises an electromagnet.

8. Apparatus according to any preceding claim, further comprising electronic control means for controlling the means for applying the magnetic field and the means for blowing the powder, the electronic control means being arranged to synchronize the application of the magnetic field with the flow of the powder.

9. Apparatus according to any preceding claim, further comprising collecting means for collecting the superconductor fine particles after they have been deflected by the magnetic field applying means.

10. Apparatus according to any of claims 1 to 8, further comprising first collecting means for collecting superconductor fine particles having a flow path deflected by the magnetic field applying means and second collecting means for collecting fine particles having a different flow path not deflected by the magnetic field applying means.

11. Apparatus according to any of claims 1 to 10, wherein the gaseous carrier medium serves as a coolant for the powder.

12. The apparatus according to any preceding claim, wherein a body of liquid is provided beneath the openings into which particles passing through the openings fall, the body of liquid serving as a coolant for the particles.

13. Apparatus according to claim 1, wherein the powder flow forming means is arranged to produce a flow of particles floated in the carrier gas, the partition means is vertically directed and is formed with a plurality of openings at different heights above the powder flow forming means, means is provided at locations facing the respective openings for applying a magnetic field to the flow of powder, and electrical control means is provided for controlling the means for forming the flow of powder and the means for applying a magnetic field.

14. Apparatus according to claim 13, wherein the means for applying a magnetic field comprises an electromagnet.

15. The apparatus of claims 13 or 14, further comprising collecting means for collecting superconductor fine particles which have travelled along the flow path and have been deflected by the magnetic field applying means.

16. Apparatus according to claim 13 or 14, further comprising first collecting means for collecting superconductor fine particles that have travelled along the flow path and have been deflected by the magnetic field applying means and second collecting means for collecting fine particles that have travelled along the flow path but have not been deflected by the magnetic field applying means.

17. The apparatus of claim 16, wherein the first collecting means and the second collecting means are controlled by the electrical control means.

18. The apparatus of any of claims 13 to 17, wherein the carrier gas serves as a coolant for the powder.

19. A method for purifying superconductor fine particles comprising:
(a) cooling the powder containing the fine particles to be purified to below its critical temperature;
(b) forming a flow of the powder along a flow path;
(c) causing the powder travelling along the flow path to enter openings at different spaced-apart locations along the path as a result of differences in the properties of the particles, and
(d) applying a magnetic field to the powder to separate the fine particles by means of their superconductivity, characterised in that:
(e) the powder flow forming means causes the powder to flow in a gaseous carrier medium along the path so that particles of different size separate according to their size and mass as they travel along the path to separate locations; and
(f) the flow of particles is caused to enter openings at different locations where gravitionally induced separation of particles of different sizes has taken place, whereby there can be obtained via the different openings purified superconductive particles having different sizes.

20. A method according to claim 19, wherein the particles are blown in a horizontal direction along a horizontal partition having slits spaced at different distances from the blowing means, and magnetic fields are applied to the particles which fall through the slits to bring about separation of the particles according to their superconductivity.

21. A method according to claim 19, wherein the powder flow forming means brings about flotation of the fine particles in an upward stream of the carrier gas, the carrier gas flows along vertically directed partition means having a plurality of slits at different heights above the flotation means, and particles of different size which separate at different heights are deflected into respective slits by magnetic field applying means which is arranged to apply a magnetic field to the powder as it flows along the partition means.

22. A method of purifying superconductive fine particles which comprises treating the particle in apparatus as claimed in any of claims 1 to 18 and recovering the purified superconductive powder.

## Patentansprüche

1. Reinigungsapparat für feine supraleitende Teilchen mit einer Einrichtung zum Abkühlen eines zu reinigenden, feine Teilchen enthaltenden Pulvers unter seiner kritischen Temperatur, einer Einrichtung (2; 32) zur Bildung eines Pulverteilchenflußes entlang einer Strecke, einer Trenneinrichtung, die eine Vielzahl von Öffnungen (11a, 11b; 34a, 34b) an unterschiedlich entfernten Stellen entlang der Strecke zum Empfangen von Teilchen mit unterschiedlichen Eigenschaften aufweist, und mit einer Einrichtung zum Anlegen eines magnetischen Feldes an den Pulverfluß, um die feinen Teilchen durch ihre Supraleitfähigkeit zu trennen, **dadurch gekennzeichnet**, **daß**
a) die Einrichtung zur Bildung des Pulverteilchenflußes so angeordnet ist, um einen Fluß des Pulvers in einem Gasträgermedium entlang der Strecke zu gewährleisten, so daß die Teilchen bei ihrer Bewegung entlang der Strecke entsprechend ihrer Größe und Masse getrennt werden; und
b) die Stellen, an denen die Öffnungen (11a, 11b; 34a, 34b) vorgesehen sind, solche Stellen sind, an denen die durch die Schwerkraft hervorgerufene Trennung von Teilchen unterschiedlicher Größe einsetzt.

2. Reinigungsapparat nach Anspruch 1, in dem die Einrichtung zur Bildung des Pulverteilchenflußes zum Ausblasen des Pulvers in horizontaler Richtung angeordnet ist, die Trenneinrichtung horizontal ausgerichtet ist und eine Vielzahl von Öffnungen in unterschiedlichen Abständen von der Einrichtung zum Ausblasen aufweist, und unter den entsprechenden Öffnungen eine Einrichtung zum Beaufschlagen des Pulvers mit einem magnetischen Feld während seiner Bewegung entlang der Strecke vorgesehen ist.

3. Reinigungsapparat nach Anspruch 2, in dem die Einrichtung zum Ausblasen eine Düse aufweist.

4. Reinigungsapparat nach Anspruch 2, in dem die Einrichtung zum Erzeugen eines magnetischen Feldes erste Magnete, die relativ dicht unter den entsprechenden Öffnungen angeordnet und auf einer ersten, relativ niedrigen Temperatur gekühlt sind, sowie zweite Magnete, die in einem relativ großen Abstand unter den entsprechenden Öffnungen angeordnet, auf einer relativ hohen Temperatur gekühlt und zum Empfangen des durch die ersten Magnete strömenden Materials vorgesehen sind, aufweist, wobei die Anordnung eine solche ist, daß nur dieses Material die zweiten Magnete durchläuft, dessen kritische Temperatur für die Supraleitfähigkeit größer ist als die zweite Temperatur.

5. Reinigungsapparat nach Anspruch 2, 3 oder 4, in dem unter einer entsprechenden Öffnung eine Prallfläche gegenüber der Ausblasrichtung des Pulvers vorgesehen ist, um das Pulver gegen die Einrichtung zum Beaufschlagen mit einem magnetischen Feld zu richten.

6. Reinigungsapparat nach einem der vorangehenden Ansprüchen, in dem die Einrichtung zum Beaufschlagen mit einem magnetischen Feld einen Permanentmagnet aufweist.

7. Reinigungsapparat nach einem der Ansprüche 1 bis 5, in dem die Einrichtung zum Beaufschlagen mit einem magnetischen Feld einen Elektromagnet aufweist.

8. Reinigungsapparat nach einem der vorangehenden Ansprüchen, mit einer elektronischen Steuereinrichtung zur Steuerung der Einrichtung zum Beaufschlagen mit einem magnetischen Feld und einer Einrichtung zum Blasen des Pulvers, wobei die elektronische Steuereinrichtung so organisiert ist, um die Beaufschlagung mit dem magnetischen Feld mit dem Pulverfluß zu synchronisieren.

9. Reinigungsapparat nach einem der vorangehenden Ansprüchen, mit einer Sammeleinrichtung zum Sammeln der feinen supraleitenden Teilchen nachdem diese durch die Einrichtung zum Beaufschlagen mit einem magnetischen Feld abgelenkt worden sind.

10. Reinigungsapparat nach einem der Ansprüche 1 bis 8, mit einer ersten Sammeleinrichtung zum Sammeln feiner supraleitenden Teilchen mit einer durch die Einrichtung zum Beaufschlagen mit einem magnetischen Feld abgelenkten Flußbahn und einer zweiten Sammeleinrichtung zum Sammeln feiner supraleitenden Teilchen mit einer unterschiedlichen, durch die Einrichtung zum Beaufschlagen mit einem magnetischen Feld nicht abgelenkten Flußbahn.

11. Reinigungsapparat nach einem der Ansprüche 1 bis 10, in dem das gasförmige Trägermedium als Kühlmittel für das Pulver dient.

12. Reinigungsapparat nach einem der vorangehenden Ansprüchen, in dem ein Flüssigkeitskörper unter den Öffnungen, in denen die durch die Öffnungen passierenden Teilchen fallen, vorgesehen ist, wobei der Flüssigkeitskörper als Kühlmittel für die Teilchen dient.

13. Reinigungsapparat nach Anspruch 1, in dem die Einrichtung zur Bildung des Pulverflußes so angeordnet ist, um einen im Trägergas schwimmenden Teilchenfluß zu erzeugen, die Trenneinrichtung vertikal ausgerichtet und mit einer Vielzahl von Öffnungen in unterschiedlichen Höhen über der Einrichtung zur Bildung des Pulverflußes ausgebildet ist, wobei eine Einrichtung an Stellen gegenüber den entsprechenden Öffnungen zum Beaufschlagen des Pulverflußes mit einem magnetischen Feld sowie eine elektrische Steuereinrichtung zur Steuerung der Einrichtung zur Bildung des Pulverflußes und der Einrichtung zum Beaufschlagen mit einem magnetischen Feld vorgesehen sind.

14. Reinigungsapparat nach Anspruch 13, in dem die Einrichtung zum Beaufschlagen mit einem magnetischen Feld einen Elektromagnet aufweist.

15. Reinigungsapparat nach Anspruch 13 oder 14, mit einer Sammeleinrichtung zum Sammeln feiner supraleitenden Teilchen, die sich entlang der Flußbahn bewegt haben und durch die Einrichtung zum Beaufschlagen mit einem Magnetfeld abgelenkt worden sind.

16. Reinigungsapparat nach Anspruch 13 oder 14, mit einer ersten Sammeleinrichtung zum Sammeln feiner supraleitenden Teilchen, die entlang der Flußbahn fortbewegt und durch die Einrichtung zum Beaufschlagen mit einem magnetischen Feld abgelenkt worden sind, und einer zweiten Sammeleinrichtung zum Sammeln von feinen Teilchen, die entlang der Flußbahn fortbewegt, jedoch durch die Einrichtung zum Beaufschlagen mit einem magnetischen Feld nicht abgelenkt worden sind.

17. Reinigungsapparat nach Anspruch 16, bei dem die erste Sammeleinrichtung und die zweite Sammeleinrichtung durch die elektrische Steuereinrichtung gesteuert werden.

18. Reinigungsapparat nach einem der Ansprüche 13 bis 17, bei dem das Trägergas als Kühlmittel für das Pulver dient.

19. Verfahren zum Reinigen feiner supraleitenden Teilchen mit den Schritten:
a) Abkühlen des Pulvers, das die feinen, zu reinigenden Teilchen enthält, unterhalb ihrer kritischen Temperatur;
b) Ausbildung eines Pulverteilchenflußes entlang einer Flußbahn;
c) Erzwingen einer Bewegung des Pulvers entlang der Flußbahn, wobei das Pulver im Ergebnis der unterschiedlichen Teilcheneigenschaften in Öffnungen, die sich entlang der Bahn an unterschiedlich entfernten Stellen befinden, eintritt, und
d) Beaufschlagen des Pulvers mit einem magnetischen Feld, um die feinen Teilchen infolge ihrer Supraleitfähigkeit zu trennen, **dadurch gekennzeichnet, daß:**
e) die Einrichtung zur Ausbildung eines Pulverflußes einen Fluß des Pulvers in einem Trägermedium entlang der Bahn hervorruft, so daß eine Trennung von Teilchen unterschiedlicher Größe entsprechend ihren Abmessungen und Masse während ihrer Bewegung zu voneinander getrennten Stellen entlang der Bahn stattfindet; und
f) der Teilchenfluß in Öffnungen an unterschiedlichen Stellen eintritt, an denen eine durch die Schwerkraft bedingte Trennung der Teilchen unterschiedlicher Größe stattgefunden hat, wodurch mittels der unterschiedlichen Öffnungen gereinigte supraleitende Teilchen unterschiedlicher Größe erhalten werden können.

20. Verfahren nach Anspruch 19, in dem die Teilchen in horizontaler Richtung entlang eines mit in unterschiedlichen Abständen von der Ausblaseinrichtung beabstandeten Spalten versehenen Trennelements geblasen werden und die Teilchen, die durch die Spalte hindurch fallen, mit magnetischen Feldern beaufschlagt werden, um eine Trennung der Teilchen entsprechend ihrer Supraleitfähigkeit zu gewährleisten.

21. Verfahren nach Anspruch 19, in dem die Einrichtung zur Ausbildung eines Pulverflußes eine Aufschwemmung der feinen Teilchen stromaufwärts des Trägergases gewährleistet, das Trägergas entlang einer senkrecht ausgerichteten Trenneinrichtung mit einer Vielzahl von in unterschiedlicher Höhe über der Aufschwemmeinrichtung befindlichen Spalten fließt, und Teilchen unterschiedlicher Größe, die in unterschiedlichen Höhen getrennt werden, in entsprechende Spalte mittels der Einrichtung zum Beaufschlagen mit einem magnetischen Feld abgelenkt werden, wobei die Einrichtung zur Beaufschlagung mit einem magnetischen Feld so angeordnet ist, um das Pulver während seines Fließens entlang der Trenneinrichtung mit einem magnetischen Feld zu beaufschlagen.

22. Verfahren zur Reinigung feiner supraleitenden Teilchen, das eine Behandlung der Teilchen in einem Apparat gemäß einem der Ansprüche 1 bis 18 sowie eine Rückgewinnung des gereinigten supraleitenden Pulvers umfaßt.

## Revendications

1. Appareil de purification de particules supraconductrices fines comprenant des moyens destinés à refroidir, au-dessous de sa température critique, une poudre devant être purifiée et contenant des fines particules, des moyens (2 ; 32) destinés à former un écoulement de la poudre le long d'un trajet, des moyens de cloisonnement ayant plusieurs ouvertures (11a, 11b ; 34a, 34b) en différents emplacements espacés le long du trajet pour recevoir des particules ayant différentes propriétés, et des moyens (5a, 5b ; 36) destinés à appliquer un champ magnétique à l'écoulement de la poudre pour séparer les fines particules au moyen de leur supraconductivité, caractérisé en ce que :
(a) les moyens formant un écoulement de poudre sont agencés de façon à amener la poudre à s'écouler dans un véhicule gazeux le long du trajet afin que des particules de différentes dimensions se séparent en fonction de leur dimension et de leur masse pendant qu'elles se déplacent le long du trajet ; et
(b) les emplacements auxquels les ouvertures (11a, 11b ; 34a, 34b) sont prévus sont des emplacements où a lieu une séparation induite par gravité des particules de différentes dimensions.

2. Appareil selon la revendication 1, dans lequel les moyens destinés à former l'écoulement de poudre sont agencés de façon à faire circuler par soufflage la poudre dans une direction horizontale, les moyens de cloisonnement sont dirigés horizontalement et présentent plusieurs ouvertures à différentes distances des moyens de soufflage, et des moyens sont prévus au-dessous des ouvertures respectives pour appliquer un champ magnétique à la poudre pendant qu'elle se déplace le long du trajet.

3. Appareil selon la revendication 2, dans lequel les moyens de soufflage comprennent une buse.

4. Appareil de purification selon la revendication 2, dans lequel les moyens produisant un champ magnétique comprennent des premiers aimants placés relativement près et au-dessous des ouvertures respectives et refroidis à une première température relativement basse, et des seconds aimants destinés à recevoir de la matière qui est passée par les premiers aimants et placés à une distance relativement plus grande au-dessous des ouvertures respectives, les seconds aimants étant refroidis à une température relativement élevée, l'agencement étant tel que seule la matière dont la température critique pour la supraconductivité est supérieure à la seconde température franchit les seconds aimants.

5. Appareil selon la revendication 2, 3 ou 4, dans lequel il est prévu, au-dessous d'une ouverture respective, un déflecteur orienté en opposition au sens dans lequel la poudre est mise en circulation par soufflage pour diriger la poudre vers les moyens d'application du champ magnétique.

6. Appareil selon l'une quelconque des revendications précédentes, dans lequel les moyens destinés à appliquer un champ magnétique comprennent un aimant permanent.

7. Appareil selon l'une quelconque des revendications 1 à 5, dans lequel les moyens destinés à appliquer un champ magnétique comprennent un électro-aimant.

8. Appareil selon l'une quelconque des revendications précédentes, comprenant en outre des moyens électroniques de commande destinés à commander les moyens destinés à appliquer le champ magnétique et les moyens destinés à faire circuler la poudre par soufflage, les moyens électroniques de commande étant agencés de façon à synchroniser l'application du champ magnétique avec l'écoulement de la poudre.

9. Appareil selon l'une quelconque des revendications précédentes, comportant en outre des moyens collecteurs destinés à collecter les particules supraconductrices fines après qu'elles ont été déviées par les moyens d'application d'un champ magnétique.

10. Appareil selon l'une quelconque des revendications 1 à 8, comportant en outre des premiers moyens collecteurs destinés à collecter des particules supraconductrices fines ayant un trajet d'écoulement dévié par les moyens d'application d'un champ magnétique et des seconds moyens collecteurs destinés à collecter des particules fines ayant un trajet d'écoulement différent, non dévié par les moyens d'application d'un champ magnétique.

11. Appareil selon l'une quelconque des revendications 1 à 10, dans lequel le véhicule gazeux sert de fluide de refroidissement pour la poudre.

12. Appareil selon l'une quelconque des revendications précédentes, dans lequel il est prévu au-dessous des ouvertures une masse de liquide dans laquelle des particules passant à travers les ouvertures tombent, la masse de liquide servant de fluide de refroidissement pour les particules.

13. Appareil selon la revendication 1, dans lequel les moyens de formation d'un écoulement de poudre sont agencés de façon à produire un écoulement de particules flottant dans le véhicule gazeux, les moyens de cloisonnement sont orientés verticalement et sont formés de plusieurs ouvertures à différentes hauteurs au-dessus des moyens de formation d'écoulement de poudre, des moyens sont prévus à des emplacements faisant face aux ouvertures respectives pour appliquer un champ magnétique à l'écoulement de poudre, et des moyens électriques de commande sont prévus pour commander les moyens destinés à former l'écoulement de poudre et les moyens destinés à appliquer un champ magnétique.

14. Appareil selon la revendication 13, dans lequel les moyens destinés à appliquer un champ magnétique comprennent un électro-aimant.

15. Appareil selon la revendication 13 ou 14, comportant en outre des moyens collecteurs destinés à collecter des particules supraconductrices fines qui se sont déplacées le long du trajet d'écoulement et qui ont été déviées par les moyens d'application d'un champ magnétique.

16. Appareil selon la revendication 13 ou 14, comportant en outre des premiers moyens collecteurs destinés à collecter des particules supraconductrices fines qui sont déplacées le long du trajet d'écoulement et qui ont été déviées par les moyens d'application d'un champ magnétique, et des seconds moyens collecteurs destinés à collecter des particules fines qui se sont déplacées le long du trajet d'écoulement, mais qui n'ont pas été déviées par les moyens d'application d'un champ magnétique.

17. Appareil selon la revendication 16, dans lequel les premiers moyens collecteurs et les seconds moyens collecteurs sont commandés par les moyens électriques de commande.

18. Appareil selon l'une quelconque des revendications 13 à 17, dans lequel le véhicule gazeux sert de fluide de refroidissement pour la poudre.

19. Procédé de purification de particules supraconductrices fines, consistant :
(a) à refroidir la poudre contenant les fines particules devant être purifiées, au-dessous de sa température critique ;
(b) à former un écoulement de la poudre le long d'un trajet d'écoulement ;
(c) à faire circuler la poudre le long du trajet d'écoulement pour qu'elle entre dans des ouvertures en différents emplacements espacés le long du trajet, par suite de différences portant sur les propriétés des particules ; et
(d) à appliquer un champ magnétique à la poudre pour séparer les fines particules au moyen de leur supraconductivité, caractérisé en ce que :
(e) les moyens de formation d'un écoulement de poudre amènent la poudre à s'écouler dans un véhicule gazeux le long du trajet afin que des particules de différentes dimensions se séparent en fonction de leur dimension et de leur masse pendant qu'elles se déplacent le long du trajet jusqu'à des emplacements séparés ; et
(f) l'écoulement de particules est amené à entrer dans des ouvertures en différents emplacements où a lieu une séparation induite par gravité de particules de différentes dimensions, grâce à quoi on peut obtenir, par l'intermédiaire des différentes ouvertures, des particules supraconductrices purifiées ayant des dimensions différentes.

20. Procédé selon la revendication 19, dans lequel les particules sont déplacées en étant soufflées dans une direction horizontale le long d'une cloison horizontale présentant des fentes espacées à différentes distances des moyens de soufflage, et des champs magnétiques appliqués aux particules qui tombent à travers les fentes pour provoquer une séparation des particules en fonction de leur supraconductivité.

21. Procédé selon la revendication 19, dans lequel les moyens formant un écoulement de poudre font flotter les fines particules dans un courant montant du véhicule gazeux, le véhicule gazeux s'écoule le long de moyens de cloisonnement orientés verticalement et ayant plusieurs fentes de différentes hauteurs au-dessus des moyens de flottation, et des particules de différentes dimensions, qui se séparent de différentes hauteurs, sont déviées dans des fentes respectives par des moyens d'application d'un champ magnétique qui sont agencées de façon à appliquer un champ magnétique à la poudre pendant qu'elle s'écoule le long des moyens de cloisonnement.

22. Procédé de purification de particules supraconductrices fines, qui comprend le traitement des particules dans un appareil selon l'une quelconque des revendications 1 à 18 et la récupération de la poudre supraconductrice purifiée.
